

No. 827,102.

S. KOHN.

PATENTED JULY 31, 1906.

PROCESS OF MANUFACTURING FIBER MATERIAL FROM ANIMAL TENDONS  
OR SINEWS.

APPLICATION FILED JAN. 19, 1906.

Fig. 1.



Fig. 2.



Fig. 3.



Fig. 5.



Fig. 4.



Witnesses:  
Wilhelm Vogt  
Thomas M. Smith.

Inventor:  
Simon Kohn,  
by  
J. Walter Douglas,  
Attorney.

# UNITED STATES PATENT OFFICE.

SIMON KOHN, OF VIENNA, AUSTRIA-HUNGARY, ASSIGNOR OF ONE-FOURTH  
TO GUSTAV POLLAK, OF VIENNA, AUSTRIA-HUNGARY.

## PROCESS OF MANUFACTURING FIBER MATERIAL FROM ANIMAL TENDONS OR SINEWS.

No. 827,102.

Specification of Letters Patent.

Patented July 31, 1906.

Application filed January 19, 1905. Serial No. 241,780.

*To all whom it may concern:*

Be it known that I, SIMON KOHN, a subject of the Emperor of Austria-Hungary, residing at the city of Vienna, in the Empire of Austria-Hungary, have invented certain new and useful Improvements in Processes of Manufacturing Fiber Material from Animal Tendons or Sinews, of which the following is a specification.

10 My invention has relation to a process for manufacturing fiber material from animal sinews or tendons, and in such connection it relates more particularly to the treatment of sinews and tendons to loosen the fiber thereof so as to render the same workable and adaptable for the manufacture of all kinds of woven and felted fabrics and of dyeing and tanning when required.

15 Heretofore an attempt was made to utilize the genital parts of bulls and oxen for the production of fibrous material therefrom. However, this object was not accomplished, as these parts are devoid of fiber, simply consisting of flesh and skin, and when treated 25 a flour or powder-like mass was obtained, which practice has demonstrated was unfit for use as a textile material in the arts.

20 The principal objects of my present invention are, first, to loosen the structure of the animal tendons or sinews by subjecting to a beating during a simultaneous turning around their longitudinal axis until the sinews or tendons have become hollow in their central portion and the bundles of the fiber mainly 25 constituting the same have been separated from each other, and, second, to completely separate the bundles of fiber located longitudinally and transversely in the sinews into finely-divided threads arranged parallel to 30 each other by a carding or combing operation.

35 The nature and scope of my invention will be more fully understood from the following description, taken in connection with the accompanying drawings, forming part hereof, 40 in which—

45 Figure 1 is an enlarged cross-sectional view of a tendon or sinew with the skin removed therefrom and illustrating the arrangement of the fiber in bundles running parallel and transversely to the longitudinal axis thereof and the albuminous cement-like substance interposed between the bundles of fibers. Fig. 2 is a perspective view of a portion of the sinew or tendon, slightly enlarged, and illus-

trating the separation of the bundles of fiber 55 from each other and from the albuminous substance and of the hollowing due to a beating simultaneously with a turning of the same around their longitudinal axis. Fig. 3 is an enlarged longitudinal sectional view of a 60 portion of the tendon or sinew shown in Fig. 2 and illustrating the bundles of fiber running in longitudinal and transverse directions and separated from each other and from the albuminous cement-like mass interposed between the fibers thereof. Fig. 4 is a side elevational view of a tendon or sinew and illustrating the partially-treated upper portion 65 and the completely-treated lower portion thereof; and Fig. 5 is a perspective view of a 70 "pizzle" which has been subjected to the same treatment as the tendon or sinew shown in Figs. 1 to 4, inclusive.

75 From the sinews or tendons are first removed all adhering flesh and fat and the skin surrounding the same. The sinews or tendons, which during the life of the animal are soft and pliable, harden shortly after death into a solid and tenaceous material, in which state the same cannot be utilized. As shown 80 in Fig. 1, the sinew A is mainly composed of parallel and transversely-arranged bundles of fibers a and b, which are separated from each other by an albuminous cement-like substance c.

85 In order to separate the bundles of fibers a and b from each other and from the substance c, the sinews or tendons A are first subjected to a beating, preferably with a hammer-like tool, (not shown,) simultaneously with a 90 turning of the same around their longitudinal axis, so that the entire surface and every point of the sinews or tendons A may be subjected to such hammer-like blows. The central portion of the tendons or sinews being of 95 somewhat less solid texture will more quickly be loosened by the hammer-like blows than the outer portions of the same, and hence the sinews or tendons will become hollow in their central portion, as shown in Fig. 2. At this 100 stage of treatment the bundles of fiber a and b, as well as the mass c, are separated from each other, as shown in Fig. 3; but the longitudinal bundles of fiber a and the transverse bundles b still keep their normal position 105 with respect to each other.

In order to bring the bundles a and b into a parallel position and to separate and finely

divide the fibers constituting the bundles, the sinews A are subjected to a carding and combing operation, by means of which the same are divided into fine and long fibers or threads d, capable of being used as a new textile material. The fiber material obtained in the above-described manner from sinews or tendons is now "roved" in the usual manner and form a fiber which may remain raw and in this state be woven and colored. Furthermore, the webs made of this fiber may be subjected to a rolling, scraping, and pressing operation, or the same may be tanned, colored, rolled, scraped, and pressed, if desired.

Having thus described the nature and objects of my invention, what I claim as new, and desire to secure by Letters Patent, is—

1. The herein-described process for manufacturing fiber material from animal tendons or sinews, which consists in first beating and simultaneously turning the sinews around their longitudinal axis and then carding to

divide the sinews or tendons into a fine thread-like material.

2. The herein-described process for manufacturing fiber material from animal tendons or sinews, which consists in first removing adhering flesh and fatty particles and the skin, then beating and simultaneously turning the sinews around their longitudinal axis to loosen the fiber bundles from each other and from the cement-like albuminous mass interposed between the same, then carding the longitudinally and transversely arranged fiber bundles to arrange the same parallel to each other so as to divide the bundles into fine thread-like material and to remove the albuminous mass therefrom.

In testimony whereof I have signed my name to this specification in the presence of two subscribing witnesses.

SIMON KOHN.

Witnesses:

WENZEL SINKERING,  
ALVESTO S. HOGUE.